

# United States Patent

[11] 3,551,727

[72] Inventors Andrew O. Jensen;  
David H. Pollock, Arcadia, Calif.  
[21] Appl. No. 646,298  
[22] Filed June 15, 1967  
[45] Patented Dec. 29, 1970  
[73] Assignee Xerox Corporation  
a corporation of New York, by mesne  
assignment

[56]

## References Cited

### UNITED STATES PATENTS

|           |         |                        |          |
|-----------|---------|------------------------|----------|
| 2,640,135 | 5/1953  | Cobine .....           | 313/311X |
| 3,098,723 | 7/1963  | Micks .....            | 313/311X |
| 3,178,308 | 4/1965  | Oxley et al. ....      | 313/341X |
| 3,201,618 | 8/1965  | Coleman .....          | 310/4    |
| 3,303,362 | 2/1967  | Webster .....          | 313/311X |
| 3,324,314 | 6/1967  | Cohen .....            | 310/4    |
| 3,376,437 | 4/1968  | Meyerand et al. ....   | 310/4    |
| 2,808,531 | 10/1957 | Katz et al. ....       | 313/346  |
| 2,986,671 | 5/1961  | Kerstetter et al. .... | 313/346  |

Primary Examiner—John W. Huckert

Assistant Examiner—Andrew J. James

Attorneys—Joseph I. Hirsch, Ronald Zibelli and Paul Enlau

[54] THERMIONIC CONVERTER HAVING A LOW  
WORK FUNCTION COLLECTOR ELECTRODE  
5 Claims, 3 Drawing Figs.

[52] U.S. Cl. .... 313/346,  
313/311; 310/4  
[51] Int. Cl. .... H01j 1/14,  
H01j 19/06  
[50] Field of Search..... 313/311,  
346; 310/4, 10, 11

**ABSTRACT:** A high temperature, low "work function" composite surface, particularly for the collector electrode of thermionic converters, which is formed by a thin layer of refractory metal containing less than 1 percent insulating metal oxide. A method of forming a high temperature, low "work function" composite surface by simultaneously vapor-depositing a refractory metal and an insulating metal oxide on a substrate.



PATENTED DEC 29 1970

3,551,727



*Fig. 1*



*Fig. 2*



*Fig. 3*

INVENTORS:  
ANDREW O. JENSEN  
DAVID H. POLLOCK

ATTORNEY:  
WILLIAM A. KEMMEL JR.

## THERMIONIC CONVERTER HAVING A LOW WORK FUNCTION COLLECTOR ELECTRODE

### BACKGROUND OF THE INVENTION

#### 1. Field of the Invention

The field of art to which the present invention pertains is broadly low work function electrodes and methods of forming them. A particular field of art in which such electrodes are used is thermionic converters.

#### 2. Description of the Prior Art

The construction and operation of thermionic converters is well known wherein a diode is formed containing a suitable vapor. The cathode or emission electrode of the diode is heated by a high temperature heat source so that electrons are emitted therefrom into the vapor to support an electrical discharge. Such electrons are then received by an anode or collector electrode and then returned to the cathode via an external electrical circuit. In effect, such device converts a portion of the heat energy supplied to the emitter electrode to electrical energy because of the difference between the high "work function" of the emitter electrode and the low "work function" of the collector electrode. As used herein, the term "work function" of the electrode may be defined simply as the energy required to completely remove an electron from the surface of the electrode. In the case of thermionic converters, the work function of the electrode is substantially determined by the character of the surface of the electrode and the vapor utilized. At present, the vapor normally used in thermionic converters is an alkali metal vapor such as cesium vapor and the electrode material is a refractory metal, usually tungsten or rhenium. Thus, a combination of cesium vapor with a rhenium collector permits high temperature operation and achieves a relatively low work function of about 1.5 electron volts for the collector, both of which are necessary for efficient operation of the thermionic converter. For example, with such collector "work function" of about 1.5 electron volts, a typical voltage output for a thermionic converter is 0.7 volts for 28 ampere per cm. load. But, if the collector "work function" can be reduced by just 0.1 electron volts, then the output voltage can be correspondingly increased by 0.1 volts and such voltage increase represents a 14 percent increase in the efficiency of the thermionic converter. Consequently, substantial research effort has been expended to produce electrode materials which will provide a low work function; however, to date, low "work function" materials have not been developed which can withstand the severe operating conditions such as are present in thermionic converters. For example, it has been found that thin films of insulated metal oxides such as aluminum oxide achieve a work function of 1.1 electron volts with cesium vapor, but such films could not be operated at high temperature, i.e., at temperatures above about 150°C.

### SUMMARY OF THE INVENTION

Consequently, an object of the present invention is a high temperature, low "work function" composite surface for electrodes. Another object of the present invention is a thermionic converter which includes a collector electrode having a high temperature, low "work function" composite surface. Still another object of the present invention is a method of forming a high temperature, low "work function" composite surface.

In general, the present invention involves a composite surface comprising a thin layer of refractory metal containing by weight less than 1 percent insulating metal oxide. The present invention also involves a collector electrode of a thermionic converter which has a composite surface comprising a thin layer of refractory metal containing by weight less than 1 percent insulating metal oxide. Finally, the present invention involves the method of forming such surface by forming a vapor deposition filament of refractory metal and positioning the surface substrate adjacent and exposed to the filament. Then a plate of insulating metal oxide is positioned adjacent and exposed to both filament and substrate. The filament is heated to evaporate the refractory metal and deposit it on the substrate

and to evaporate and deposit a portion of the insulating metal oxide with the refractory metal on the substrate.

### BRIEF DESCRIPTION OF THE DRAWING

5 In order to facilitate understanding of the present invention reference will now be made to the appended drawing of a preferred specific embodiment of the apparatus used in the method of the present invention. Such drawing should not be construed as limiting the invention, which is properly set forth in the appended claims. In the drawings:

10 FIG. 1 is a cross-sectional view of the specific embodiment of the apparatus used in the method of the present invention shown in FIG. 2 taken along the line 1-1 of FIG. 2.

15 FIG. 2 is a cross-sectional view of the apparatus shown in FIG. 1 taken along line 2-2 of FIG. 1.

20 FIG. 3 is a cross-sectional view of a thermionic converter constructed according to this invention.

### DESCRIPTION OF THE PREFERRED EMBODIMENT

The present invention involves in its broadest aspects a high temperature, low "work function" composite surface comprising a thin layer of refractory metal containing by weight less than 1 percent insulating metal oxide. Such layer should be less than 0.01 inches thick and preferably have a thickness in the range of about 0.0005 inches to 0.002 inches. Refractory metals which may be used in the composite surface include rhenium, tungsten, molybdenum, tantalum, with rhenium being preferred. The insulating metal oxide which may be used in the composite surface include aluminum oxide, beryllium oxide, and magnesium oxide, with aluminum oxide being preferred. The concentration by weight of the insulating metal oxide in the refractory metal layer should be less than 1 percent and is, preferably, in the range of about 0.10 percent to 0.20 percent. The composite surface should be formed as a layer on a suitable refractory metal substrate such as molybdenum.

25 A specific application of the above described composite surface is in a thermionic converter having an emitter electrode, a collector electrode, and a vapor contained between such electrodes and adapted to support an electrical discharge therebetween. In such thermionic converter, a collector electrode having the above described composite surface and comprising a thin layer of refractory metal and containing by weight less than 1 percent insulating metal oxide, provides a substantially improved performance, i.e., the voltage output and operating efficiency of the thermionic converter are substantially increased.

30 The method of forming the high temperature, low "work function" composite surface of the present invention is illustrated by the apparatus shown in FIGS. 1 and 2. As shown therein, the apparatus 10 includes a flat coil 11 of rhenium with its leads 12 extending perpendicular to the plane of the coil 11 and to the rear of the coil 11. The coil 11 is supported by its leads 12 being mounted on and extending through a plate 13 of aluminum oxide positioned adjacent to and parallel to the coil 11. Mounted on the plate 13 by struts 14 is an inner

35 cylindrical tantalum shield 15 which extends parallel to the leads 12 and surrounds the leads 12 and coil 11. The coil 11, leads 12, plate 13, and inner shield 15 are in turn mounted within an outer cylindrical tantalum shield 16 by attaching the plate 13 to the outer shield 16 by tabs 17. The substrate 20 to be coated by the apparatus 10 is positioned adjacent and parallel to the coil 11 on the opposite side of the plate 13, i.e., at the front of the coil 11.

40 Thus, the method of forming the composite surface of the present invention involves forming a vapor deposition filament of a refractory metal such as coil 11. Then, the surface substrate 20 is positioned adjacent and exposed to such filament. Also, a plate 13 of insulating metal oxide is positioned adjacent and exposed both to the filament 11 and the substrate 20. Finally, the filament 11 is heated to evaporate and deposit both the refractory metal and the insulating metal

45 50 55 60 65 70 75

oxide on the substrate 20 so that a composite surface is deposited on the substrate.

A specific example of the method and composite surface of the present invention involves positioning a molybdenum substrate approximately one-eighth inch from one side of a rhenium coil and an aluminum oxide plate approximately one-half inch from the opposite side of said coil. The coil is then heated in a vacuum to 2,700°C. for about one-half hour. The resulting rhenium film deposited on a molybdenum substrate had a thickness of approximately 0.001 inches and contained approximately 0.13 percent aluminum oxide by weight. Such composite surface was then tested by including the surface into an electron emission test vehicle. The results of such testing showed that the composite surface exhibited a work function of 1.2 electron volts. For comparison, a rhenium metal surface was formed under the same conditions except the aluminum oxide plate was absent so that there was no resulting aluminum oxide in the deposited surface. The resulting measured work function was 1.5 electron volts.

In FIG. 3 there is shown a thermionic converter 21. The thermionic converter 21 includes a collector electrode 22 having the above described composite surface, an emitter electrode 23 spaced apart from the collector electrode and a vapor 24 contained in the space between the collector electrode 22 and the emitter electrode 23 and adapted to support an electrical discharge therebetween.

There are a number of features of the present invention which clearly show the significant advance the present invention represents over the prior art. However, only a few of the more outstanding features will be pointed out to illustrate the unexpected and unusual results obtained by the present invention. One feature of the present invention is the high temperature, low "work function" composite surface which may be used on the collector electrode of a thermionic converter and which is stable despite the severe operating conditions to which it is subjected. Because of such feature, a substantial in-

crease in the voltage output and efficiency of the thermionic converter may be achieved. Another feature of the present invention is the simple method of forming the composite surface of the present invention wherein vapor deposition is utilized not only to deposit the refractory metal layer but also to generate and deposit the insulating metal oxide portion of such layer.

It will be understood that the foregoing description and example are only illustrative of the present invention and it is not intended that the invention be limited thereto. All substitutions, alterations, and modifications of the present invention which come within the scope of the claims or to which the present invention is readily susceptible without departing from the spirit and scope of this disclosure are considered part of the present invention.

We claim:

1. In a thermionic converter comprising an emitter electrode, a collector electrode and a vapor contained between said electrodes and adapted to support the electrical discharge therebetween, the improvements comprising a collector electrode having a composite surface, comprising a thin layer of refractory metal containing by weight less than 1 percent of an insulating metal oxide.

2. A thermionic converter as stated in claim 1 wherein said layer is less than about 0.01 inches thick.

3. A thermionic converter as stated in claim 1 wherein said refractory metal is rhenium.

4. A thermionic converter as stated in claim 1 wherein said insulating metal oxide is aluminum oxide.

5. A thermionic converter as stated in claim 1 and wherein the refractory metal is rhenium, the insulating metal oxide is aluminum oxide and the concentration by weight of the aluminum oxide is in the range of about 0.10 percent to 0.20 percent.

40

45

50

55

60

65

70

75